# EUROPEAN PATENT APPLICATION

(11) **EP 0 104 260 A1**
(43) Date of publication of application: **04.04.1984**
(21) Application number: 83901099.8
(22) Date of filing: 31.03.1983
(51) Int. Cl.: B41J 3/10

(54) **WIRE FOR DOT PRINTER**

(30) Priority: 01.04.1982 JP 54082/82
(71) Applicant: HITACHI METALS, LTD., Chiyoda-ku, Tokyo 100 (JP)
(72) Inventor: SAKAKIBARA, Masahiko, Saitama 360 (JP)
(74) Representative: Strehl, Peter, Dipl.-Ing.
(86) International application number: JP8300102
(87) International publication number: WO8303385

(57) **Abstract**

Improvement in a wire for a dot printer. The wire is made of a very tough base metal with a very hard, highly wear-resistant film coated onto the base metal. The conventional wire of this type has the technical problem that irregular wear is produced when it is used in a dot printer, this problem is eliminated by covering the base metal with the film.

## Description

### TECHNICAL FIELD

The present invention relates to an improvement in wire for use in dot printer and, more particularly, to an improvement in the wear resistance of such wire.

### BACKGROUND ART

Figs. 1 and 2 show an example of printhead for dot printer which is presently used ordinarily. More specifically, Fig. 1 is a sectional view, while Fig. 2 is an exploded perspective view of the printhead.

In Figs. 1 and 2, a reference numeral 1 denotes a first plate forming a common magnetic path, 2 denotes a plurality of cores fixed to the plate 1, 3 denotes a ring-shaped permanent magnet fixed to the plate 1, 4 denotes magnet coils fitted to respective cores 2, 5 denotes a second plate forming a common magnetic path and provided with holes 5a at positions corresponding to the cores 2, 6 denotes a spacer, 7 denotes a leaf spring having one end connected in a ring-like form and having holes 7a corresponding to the holes 5a of the second plate 5 and slitted at the end 7b into sections which are deflectable independently, 8 denotes a wire fixed to the end 7b of the leaf spring 7 by, for example, brazing, 9 denotes armature pins fitted in the holes 7a in the leaf spring 7 and opposing to the holes 5a in the plate 5 and also to the cores 2, 10 denotes a guide frame, and 11 denotes a pin guide mounted on the end of the guide frame 10. The guide frame 10 and the pin guide 11 in combination constitutes a guide member.

In operation, when the magnet coils 4 are not energized, the armature pins 9 on the end 7b of the leaf spring 7 are attracted to the cores 2 by the magnetic force of the permanent magnet 3. In this state, therefore, the end 7b of the leaf spring 7 is biased. Then, as one of the magnet coils 4 is energized, the magnetic field produced by the magnet coil 4 cancels the magnetic field of the permanent magnet 3, so that the armature pin 9 on the leaf spring 7 is freed from the attracting force produced by the core 2. Consequently, the end 7b of the leaf spring 7 is relieved from the biasing force, so that the wire 8 fixed to the end of the leaf spring 7 is driven while being guided by the pin guide 11. As the magnet coil 4 is de-energized, the armature pin 9 on the leaf spring 7 is attracted again to the core 2 by the magnetic force of the permanent magnet 3.

In the prithead H of the dot printer of the kind described, a plurality of wires are guided by the pin guide 11 and the arrayed substantially in a linear line. However, the base end portions of the wires fixed to the leaf spring 7 are arranged substantially along an oval line, so that the wire is obliged to be slightly inclined to the print surface when printing. Partly because of this reason, as well as for other reasons, a local wear of the wire end surface inevitably takes place as a result of repeated printing action,. resulting in a vagueness of the printed characters.

As a measure for overcoming the above-described problem of the prior art, it has been proposes to use wire made from a super hard alloy or ceramics material. These materials, however, suffers from various shortcomings such as small impact strength and inferior weldability which makes it difficult to fix them to the leaf spring, although they exhibits a high wear resistance. Under this circumstance, there is an increasing demand for a wire for use in dot printer improved to overcome these problems of the prior art.

### DISCLOSURE OF THE INVENTION

In order to cope with the above-described demand, the present invention aims as its major object at providing a wire for use in dot printer having a superior impact strength and exhibiting a high resistance to local wear.

To this end, according to the invention, there is provided a wire for use in dot printer having a base member constituted by a metallic material and a hard coating film of ceramics on the base member so that a high toughness and small local wear are ensured by the toughness inherent in the metallic material and high wear resistance peculiar to the ceramics material.

According to the invention, it is possible to use, as the metallic material of the base member, various materials known as the material of the wire for use in dot printer, such as high-speed tool steel, die steel, other tool steels, tungsten steel, piano wire and so forth. Among these known materials, the high-speed tool steel can be used most suitably as the material of the base member of the wire for use in dot printer of the invention, because it exhibits a high flexural toughness and large deflective strength, as well as good brazing characteristic.

Further, in the present invention, as the hard coating film, it is possible to use various coating materials known as hard coating materials, such as carbides, nitrides, borides, oxides, carbonitrides and other compounds of various metallic elements. A good results is obtained particularly when ceramics coating film such as of TiC, TiN, TiCN, TiB₂, VC, Al₂0₃ and the like are used.

As to the thickness of the coating, an appreciable effect is obtained even when the coating film thickness is less than 1 µm, but since a better property is obtained when the coating film thickness is in a range between 1 and 10 pm, the thickness in this range is preferable. Although the structure of the coating film is selector in accordance with the materials of the base member and the coating film, it is needless to say that the coating film may be composed of a single layer or a multiplicity of layers.

According to the invention, the adhesion or affinity between the base member and the coating film is a matter of great significance. Therefore, the coating film is made preferably by chemical deposition method (CVD method), molten salt method, ion-plating method or the like.

### BRIEF DESCRIPTION OF THE DRAWINGS

Figs. 1 and 2 are a sectional view and an exploded perspective view of the printhead for a dot printer; and
Fig. 3 is a microscopic photo of the cross- section of coating film of a wire for use in dot printer in accordance with the invention.

### THE BEST MODE FOR CARRYING OUT THE INVENTION

The invention will be described in detail hereinunder through an embodiment.

A wire for use in dot printer made from a high-speed tool steel was cleaned and sufficiently degreased in a triqhlene bath under application of a ultrasonic cleaning. The wire thus treated was placed in an ion-plating apparatus. At the same time, metallic Ti having purity of 99.9 % or higher as the evaporation material was set in the same. After evacuating the inside of the apparatus to a high vacuum exceeding 10⁻⁵ Torr, the vacuum was decreased to 5 x 10⁻⁴ Torr by introduction of argon gas and then to 1 x 10⁻³ Torr by introduction of nitrogen gas.

Then, D.C. voltage of 2 KV was applied to the electrically insulated wire holder to cause an electric discharge and, at the same time, the metallic Ti was heated and evaporated by the application of electron beam. This condition was maintained for about 15 minutes to form a TiN coating film of 1.5 pm thick on the wire. A wire for use in dot printer made of high-speed tool steel and having a TiN coating film was thus produced. Fig. 3 shows a microscopic photo of the cross- section of the coating film of this wire for use in dot printer. From this Figure, it will be seen that the coating film covers the base member with a high affinity or adhesion.

For a comparison, a conventional wire for use in dot printer made of high-speed tool steel having no TiN coating film was produced. Table 1 shows the properties of the wire for use in dot printer of the invention in comparison with those of the conventional wire for use in dot printer.

A practical wear resistance test was conducted with the wire of the invention which has been subjected to the TiN coating treatment and the conventional wire. As a result, the dot printer using conventional wire showed a local vagueness of the print after a long use on the order of 1,000 hours. In contrast, the dot printer using the wire of the invention did not show any substantial degradation in the clearness of the print even after the use for about 4,000 hours.

From this test result it is clear that the invention provides a distinctive effect in improving the wear resistance of the wire for use in dot printer. In addition, the wire in accordance with the invention showed a good brazing characteristic, so that it could be fixed to the leaf spring easily and securely.

As has been described, the invention makes it possible to provide a wire for use in dot printer which can stand much longer use than the conventionally used wire for use in dot printer. Thus, the invention offers a great advantage from the industrial point of view.

## Claims

1. A wire for use in dot printer comprising a metallic wire and a hard coating film formed on the surface of the metallic wire.

2. A wire for use in dot printer according to claim 1, wherein said hard coating film has a hardness of Hv 1,000 or higher.

3. A wire for use in dot printer according to claim 1 or 2, wherein said hard coating film has a thickness ranging between 1 and 10 µm.

4. A wire for use in dot printer according to claim 1, 2 or 3, wherein said hard coating film is constituted by one, two or more selected from the group consisting of TiC, TiN, TiCN, TiB₂, VC and Al₂O₃.

1. A wire for use in dot printer comprising a high-speed tool steel wire and a hard coating film formed on the surface of the high-speed tool steel wire.

2. A wire for use in dot printer according to claim 1, wherein said hard coating film has a hardness of Hv 1,000 or higher.

3. A wire for use in dot printer according to claim 1 or 2, wherein said hard coating film has a thickness ranging between 1 and 10 µm.

4. A wire for use in dot printer according to claim 1, 2 or 3, wherein said hard coating film is constituted by one, two or more selected from the group consisting of TiC, TiN, TiCN, TiB₂, VC and A1₂0₃.
